

1

3,829,311

## ADDITION ALLOYS

John William Grant, Radlett and Gordon John Cox, Sutton Coldfield, England, assignors to The International Nickel Company, Inc., New York, N.Y.

No Drawing. Filed Sept. 11, 1972, Ser. No. 287,880  
Claims priority, application Great Britain, Sept. 9, 1971,  
42153/71

Int. Cl. C22c 29/00

U.S. CL. 75—122

6 Claims

## ABSTRACT OF THE DISCLOSURE

Directed to alloys which are particularly suitable for the introduction of magnesium into molten iron and which contain in weight percent about 5% to 15% nickel, about 5% to 14% magnesium, about 34% to 60% silicon, about 0.5% to about 3% of a rare earth metal, up to about 4% calcium, up to about 2% carbon, up to about 10% manganese, up to about 10% copper, the balance being essentially iron, in an amount less than about 50%.

This invention is directed to alloys and, in particular, to addition alloys suitable for the introduction of magnesium into molten iron.

The introduction of magnesium into molten iron is widely known and practiced for the production of spheroidal graphite cast iron in which the graphite is rendered spheroidal by means of retained magnesium. To insure that the graphite formed in the cast iron, either on solidification, or during a graphitizing heat treatment, is spheroidal, generally requires a retained magnesium content of up to about 0.1%, e.g., from 0.02% to 0.08%.

As is well known in the art, the direct addition of magnesium metal to molten metal is generally not practiced because of its high vapor pressure of about 6 to 10 atmospheres at the usual temperature of treatment, for example, 1400° C. to 1500° C.; at these conditions, there would be a violent reaction. Several processes have been developed to add magnesium safely to the molten metal, one of which is the use of addition alloys.

Of the addition alloys employed at present, those containing nickel are extremely effective in moderating the violence of the reaction between the magnesium and molten iron. It has generally been found however, that large percentages of nickel, e.g., 60% to 70% or more are necessary in order that a high alloy efficiency may be obtained. The utility of an addition alloy for introducing magnesium into molten metal is measured in terms of its efficiency and it is essential that a high alloy efficiency be obtained because at lower efficiencies more alloy must be added to the molten metal to introduce the desired quantity of magnesium. The introduction of large quantities of addition alloy to the melt may cause additional problems because of excessive cooling and can result in an increased tendency for the occurrence of dross and other casting defects. As in all commercial processes, it is also essential that the additional alloys be economical to use.

It is an object of the present invention to provide addition alloys for use in introducing magnesium to molten iron which possess high cost efficiencies, that is, optimum magnesium recovery coupled with lowest addition alloy cost.

Generally speaking, the present invention is directed to alloys containing (in weight percent) about 5% to about 15% nickel, about 5% to about 14% magnesium, about 34% to about 60% silicon, about 0.5% to about 3% of a rare earth metal, up to about 4% calcium, up to about 2% carbon, up to about 10% manganese, up to about 10% copper, and the balance essentially iron, the iron content being less than about 50%.

2

In carrying the invention into practice, a preferred compositional range comprises about 8% to about 15% nickel, about 9% to about 13% magnesium, about 34% to about 50% silicon, about 1.5% to about 2.5% of a rare earth metal, about 1.5% to about 2.5% calcium, the balance being essentially iron.

A more preferred alloy comprises about 9% to about 13% nickel, about 9% to about 13% magnesium, about 38% to about 45% silicon, about 1.5% to about 2.5% of a rare earth metal, about 1.5% to about 2.5% calcium, up to about 1% carbon and the balance essentially iron.

As described above, the utility of an addition alloy for introducing magnesium into molten metal may be measured in terms of its efficiency, which may be defined as follows:

Efficiency (percent)

$$\frac{\text{Mg recovery (percent)} \times \text{Mg content of alloy (percent)}}{100}$$

20 where:

Mg recovery (percent)

$$25 = \frac{\left( \text{Residual Mg (percent) in the iron} + \frac{3}{4} \text{ (initial sulfur content of the iron (percent))} \right)}{\text{Mg added (percent) to the iron}} \times 100$$

It is essential that the nickel content be at least 5% for acceptable magnesium recovery and consequently, acceptable alloy efficiency. Nickel contents below 5% in the alloy result in sharp reduction of these properties 30 therein, while nickel contents exceeding about 15% add to the cost of the alloy. For maximum cost-efficiency, the preferred nickel content is at least 8% but less than about 15%, and most preferably is from 9% to 13%.

Alloys containing less than about 5% magnesium provide excellent recovery values but, because there is a low magnesium content, the efficiency is poor. If the alloys contain more than about 14% magnesium, undesirably increased reactivity may be experienced on addition of the alloy to molten iron resulting in a low magnesium recovery and hence, inadequate efficiency. For optimum efficiency a magnesium content of from about 35 9% to about 13% is preferred.

Silicon is essential in the alloy to ensure that the melting point of the alloy is low compared with the normal temperatures encountered in handling molten iron in the foundry. If the melting point of the alloys is high, e.g., about 1450° C., the alloys are difficult to produce and difficult to melt in the molten iron to which they are 40 added. The presence of silicon in the alloy in amounts from about 34% to about 60% reduces the melting point of the alloy to a temperature which is low in relation to the usual handling temperature of molten iron in the foundry and, in addition, results in the need for a smaller 45 amount of ferro-silicon graphitizing inoculant, which is commonly employed as a late addition in the manufacture of spheroidal graphite iron. However, at higher pouring temperatures, for example, 1480° C. and above, the magnesium recovery tends to decrease at high silicon 50 levels. For this reason and for greater ease of manufacture it is preferred that the silicon content of the alloy be maintained from about 34% to about 50%, and more preferably, from about 38% to about 45%.

The presence of rare earth metals in the alloy raises 55 the magnesium recovery of the alloy. The rare earth metals are also beneficial in offsetting the effect of incidental elements which may be present in the base charge and which may interfere with the formation of spheroidal graphite. One or more of the rare earth elements may be added, for example, in the form of Mischmetal, in an amount of at least 0.5%. The rare earth metal content of the alloy can be extended up to about 3% but at 60

about this level and above no additional benefits are conferred. It is most preferred that the total rare earth metal content be from about 1.5% to about 2.5%.

Calcium in the alloy also contributes to magnesium recovery. For this purpose at least 0.5% may be employed in the alloy, but amounts of calcium in excess of about 4% provide no further benefits. Calcium also produces the beneficial effect of reducing the violence of the addition reaction. It is most preferred that the content of calcium in the alloy be from about 1.5% to about 2.5% or about 3%.

Carbon may be present in the alloys in amounts up to about 2%. It is believed that this element confers the advantage of reducing the violence of the reaction when the alloys are added to molten iron. A range of about 0.1% to about 1% is beneficial. The alloy may also contain up to about 10% manganese and up to about 10% copper without adversely affecting their general properties. It is preferred however, that both manganese and copper contents not exceed about 5%.

The balance of the composition, up to about 50%, is iron, including small amounts of impurities. The presence in the alloy of iron exceeding about 50% can lead to an excessively high alloy melting point, which causes addition alloy production and melting difficulties.

The nickel-containing alloys of the invention are characterized by the presence of three phases, namely a silicon-magnesium phase in a matrix comprising iron-silicon and nickel-silicon phases. Electron microprobe analysis of the silicon-manganese phase revealed a high silicon to manganese ratio of 8.1:1 by weight.

The alloys contemplated in the present invention may be processed following normal operating procedures. They may be readily added to an iron or other molten melt either by throwing the alloy onto the melt or by placing the alloy in an empty vessel and pouring the melt onto it. For best results, it has been found that a method of addition known as the "sandwich method" is the most advantageous. In this method, the bottom of a ladle is built up over approximately half its area, for example, by 10 cm. The addition alloy is then placed against the ledge thus formed and covered with mild steel clippings, which usually comprise about 2% by weight of the metal to be treated. The melt is then tapped onto the platform and allowed to flow over the clippings and addition alloy.

In order to give those skilled in the art a better understanding of the invention, the following examples are given:

TABLE I

| Alloy | Composition (percent) |      |       |            |       |       |       |       |
|-------|-----------------------|------|-------|------------|-------|-------|-------|-------|
|       | Ni                    | Mg   | Si    | Rare earth | Ca    | C     | Al    | Fe    |
| 1     | 11.2                  | 9.7  | 38.3  | 2.16       | 2.2   | 0.44  | ----- | Bal.  |
| 2     | 11.4                  | 10.0 | 34.8  | 2.35       | 3.0   | 0.66  | ----- | Bal.  |
| 3     | 10.95                 | 11.0 | 49.5  | 2.4        | 2.8   | 0.19  | ----- | Bal.  |
| 4     | 6.0                   | 6.9  | 42.1  | 2.16       | 2.1   | 0.21  | ----- | Bal.  |
| A     | Bal.                  | 15.9 | ----- | 0.46       | ----- | 1.5   | ----- | ----- |
| B     | -----                 | 10.7 | 47.4  | 1.16       | ----- | 0.096 | 1.0   | 42.0  |

10 Addition alloys 1 to 4 were then employed in the production of S.G. iron by the "sandwich method." A charge of pig iron containing 3.8% carbon, 0.1% silicon, 0.025% phosphorus and 0.01% sulfur was melted in a 100 kg. basic HF furnace for use with each 15 addition alloy and the silicon content of the melt was adjusted by the addition of ferro-silicon. The temperature was raised 1450° C., a small addition of manganese was made and the melt was poured at 1450° C. into a ladle containing the addition alloy. The addition alloy (0.8% by weight of the total melt) was placed against a shelf 20 in a ladle and covered with mild steel clippings (2% by weight of the total melt), and the molten iron was poured onto the shelf. Finally the melt was inoculated with ferro-silicon. Spheroidal graphite iron was produced in a similar manner using Alloys A and B. One 30 mm. x 35 mm. x 165 mm. keel block was cast from each melt together with one analysis sample. The compositions of the spheroidal-graphite irons are given in Table II together with performance data calculated for each of the alloys.

TABLE II

| Addition alloy | S.G. iron composition, percent |      |      |       | Alloy performance  |                      |
|----------------|--------------------------------|------|------|-------|--------------------|----------------------|
|                | Si                             | Mn   | Ni   | Mg    | Mg                 | Alloy                |
|                |                                |      |      |       | (percent) recovery | (percent) efficiency |
| 1              | 2.00                           | 0.51 | 0.14 | 0.037 | 57.2               | 5.5                  |
| 2              | 2.90                           | 0.52 | 0.10 | 0.038 | 56.9               | 5.7                  |
| 3              | 2.05                           | 0.50 | 0.11 | 0.044 | 58.4               | 6.4                  |
| 4              | 1.90                           | 0.54 | 0.26 | 0.031 | 69.0               | 4.8                  |
| A              | 1.50                           | 0.4  | 0.37 | 0.036 | 66.5               | 10.6                 |
| B              | 1.40                           | 0.4  | 0.02 | 0.032 | 29.2               | 3.1                  |

## EXAMPLE II

Alloy performance tests similar to the one described in Example I, except that the pouring temperature is 45 1480° C., were conducted using Alloys 3 and B, described hereinabove in Table I, and Alloy 5 which contained 10.6% nickel, 11.2% magnesium, 38.2% silicon, 2.7% rare earth metal, 1.24% calcium, 1.12% carbon and the balance essentially iron. The data are given in Table III.

TABLE III

| Test No. | Addi-<br>tion<br>alloy | Amount<br>added,<br>percent | S.G. iron<br>composition, percent |      |      |       | Alloy performance            |                                  |
|----------|------------------------|-----------------------------|-----------------------------------|------|------|-------|------------------------------|----------------------------------|
|          |                        |                             | Si                                | Mn   | Ni   | Mg    | Mg<br>(percent)<br>recovery* | Alloy<br>(percent)<br>efficiency |
| 1        | 3                      | 0.8                         | 2.21                              | 0.51 | <0.1 | 0.032 | 41.5                         | 4.6                              |
| 2        | B                      | 1.2                         | 2.45                              | 0.28 | <0.1 | 0.018 | 22.4                         | 2.4                              |
| 3        | 5                      | 0.9                         | 2.32                              | 0.18 | <0.1 | 0.039 | 57.6                         | 6.4                              |

\* S content before treatment was 0.006% for Test No. 1, 0.015% for Test No. 2 and 0.025% for Test No. 3.

## EXAMPLE I

The addition alloys (1 to 4) of the compositions shown hereinbelow in Table I were all prepared in a basic HF induction furnace by adding the various elements to a base iron-silicon melt maintained at 1150° C. Quiescent melting of these additions was obtained by plunging them through a cover of crushed graphite. After the additions the temperature was raised to about 1240° C. and the graphite cover removed. The melt was then tapped into metal slab molds, 30 cm.<sup>2</sup> and 5 cm. thick. Alloys A and B are not in accordance with the invention.

65 Further tests in which various amounts of addition alloys of the invention were added to iron melts reveal the surprising effect that the magnesium recovery increases with decreasing additions of addition alloy. This makes it possible to achieve a given residual magnesium content 70 by the use of smaller amounts of addition alloy with the resulting benefits of minimizing cooling effects and increasing cost efficiency.

A nickel-free alloy containing 9.6% magnesium, 48.7% silicon and the balance iron, i.e., similar to Alloy B in 75 Table II, contained only iron-silicon and silicon-magne-

sium phases, the proportion of the silicon-magnesium phase being appreciably less than in Alloy No. 1 (9.7% magnesium and 38.3% silicon) and the ratio of silicon to magnesium within this phase being 0.9:1. The magnesium recovery value obtained for the latter alloy under the conditions employed in Example I was only 26.7%, compared with 57.2% for Alloy No. 1 the structure of which was found to comprise a silicon-magnesium phase in a matrix of iron-silicon and nickel-silicon phases, the silicon-magnesium phase having a silicon to magnesium ratio of 8.1:1. These results suggest that the magnesium recovery increases with an increasing silicon to magnesium ratio in the silicon-magnesium phase of the addition alloy.

Although the present invention has been described in conjunction with preferred embodiments, it is to be understood that modifications and variations may be resorted to without departing from the spirit and scope of the invention, as those skilled in the art will readily understand. Such modifications and variations are considered to be within the purview and scope of the invention and appended claims.

We claim:

1. An alloy consisting essentially of about 5% to about 15% nickel, about 5% to about 14% magnesium, about 34% to about 60% silicon, about 0.5% to about 3% rare earth metal, about 0.5% to about 4% calcium, up to about 2% carbon, up to about 10% manganese, up to

about 10% copper and the balance essentially iron, with the iron less than about 50%.

2. An alloy in accordance with claim 1 wherein the carbon does not exceed about 1%, the manganese does not exceed about 5% and the copper does not exceed about 5%.

3. An alloy in accordance with claim 1 wherein the rare earth metal is in the form of Mischmetal.

4. An alloy in accordance with claim 1 wherein the nickel is about 8% to about 15%, the magnesium is about 9% to about 13%, the silicon is about 34% to about 50%, the rare earth metal is about 1.5% to about 2.5% and the calcium is about 1.5% to about 2.5%.

5. An alloy in accordance with claim 4 wherein the nickel is about 9% to about 13% and the silicon is about 38% to about 45%.

6. An alloy in accordance with claim 5 wherein the carbon does not exceed about 1%.

20

#### References Cited

#### UNITED STATES PATENTS

|           |        |         |       |        |
|-----------|--------|---------|-------|--------|
| 3,295,963 | 1/1967 | Galvin  | ----- | 75—122 |
| 3,033,676 | 5/1962 | Cox     | ----- | 75—122 |
| 3,304,174 | 2/1967 | Ototani | ----- | 75—122 |
| 3,715,206 | 2/1973 | Komatsu | ----- | 75—122 |

HYLAND BIZOT, Primary Examiner

5

10

15

20

25

UNITED STATES PATENT OFFICE  
CERTIFICATE OF CORRECTION

PATENT NO. : 3,829,311  
DATED : August 11, 1974

INVENTOR(S) : JOHN WILLIAM GRANT and GORDON JOHN COX

It is certified that error appears in the above-identified patent and that said Letters Patent are hereby corrected as shown below:

Column 1, line 59, for "additional" read --addition--.

Column 3, line 30, for "manganese" read --magnesium--.

Column 4, line 18, after "raised", insert --to--.

Column 4, line 57, for "Amount" read --Amounts--.

Signed and Sealed this

Twenty-first Day of September 1976

[SEAL]

Attest:

**RUTH C. MASON**  
*Attesting Officer*

**C. MARSHALL DANN**  
*Commissioner of Patents and Trademarks*